

## UNITED STATES PATENT OFFICE.

LINDOLPH MINOR SHEROW, OF OSSINING, NEW YORK.

## COMPOSITION OF MATTER FOR SILVERPLATING METALS.

No Drawing.

Application filed June 6, 1922. Serial No. 566,411.

*To all whom it may concern:*

Be it known that I, LINDOLPH MINOR SHEROW, a citizen of the United States, and residing at Ossining, in the county of West Chester and State of New York, have invented a certain new and useful Composition of Matter for Silverplating Metals, of which the following is a specification, such as will enable those skilled in the art to which it appertains to make and use the same.

This invention relates to compositions of matter and particularly to a silver plating solution, paste or powdered substance adapted to be applied to a piece of metal for giving such metal a silver plating or coating; and the object of the invention is to provide a composition of the class specified which will polish the metal surface to which it is applied and also form a silver plating or coating thereon; and with this and other objects in view the invention consists in a combination of the class and for the purpose specified made in the manner hereinafter described and claimed.

In carrying my invention into effect, I employ the following ingredients which are combined in the manner hereinafter set out.

Pure silver metal,  
Nitric acid,  
30 Camphor gum,  
Peroxide of hydrogen solution (or double distilled water),  
Sodium cyanide,  
Paris white,  
35 Oil of mirbane.

In practise camphor gum is dissolved in peroxide of hydrogen solution, or in water, to such an extent that the peroxide of hydrogen solution or water will take up the 40 camphor to make a camphorated peroxide or water solution.

In making up a quantity of this substance I take four hundred and eighty grains of the silver crystal (silver nitrate) and dissolve 45 the same in two quarts of the camphorated peroxide solution, this is done in one vessel or vat and in another vessel or vat, I dissolve one and one-quarter pounds of sodium cyanide in eight quarts of the camphorated 50 peroxide or water solution. When both of these solutions are thoroughly mingled and dissolved I pour the first named or silver solution into the second named or sodium cyanide solution thoroughly stirring or agitating the solutions during this operation, after 55 which ten pounds of Paris white into which

two teaspoonsful of oil of mirbane have been absorbed is stirred into the solution to form my improved silver plating or coating solution.

A solution made in the manner above set out if applied to a rag or the like and rubbed upon a piece of metal to be cleaned and plated, the solution will first clean the surface, if cleaning be necessary, after which it will leave a plating or coating of silver on such surface. One application of the solution will be all that is necessary, but if more than one application is used a stronger plating or coating will be produced. In 70 the use of my improved product, it is necessary to agitate or shake the solution immediately before using as a deposit will be present in the bottom of the container in which the solution is placed.

My improved cleaning and plating solution may be put up in a small flask at a comparatively reasonable price and will apply a plating or coating of silver to a metal surface which will remain bright and of a 80 silvery appearance for a considerable length of time without tarnishing or discoloring.

My improved solution is designed particularly for use in plating various ornametal, decorative or finished metalware, but may 85 also be used in plating silver flat-ware, including forks, knives, spoons and the like, if desired, and particularly in plating silver-plated ware and will operate to materially lengthen the life of plated ware of this 90 class.

My improved composition may also be made up in the form of a paste-like substance by simply allowing the water or peroxide of hydrogen solution to evaporate or 95 partially evaporate, and this paste-like substance may be put up in jars or other containers and may be applied with a damp cloth as will be apparent.

I may also make up my improved product in the form of a powder in which event the silver nitrate in a crystal form is ground into a powder as is also camphor gum and sodium cyanide, and these products are mingled with Paris white in the proportions 105 above named, to form a powdered substance which may be rubbed onto a piece of metal to be plated, but preferably by the use of a damp cloth.

It will be understood that I am not necessarily limited to the specific proportions 110 of the various ingredients herein described,

nor am I necessarily limited to the specific ingredients herein set out, as any other ingredients having the same active properties may be substituted for those named, as for example, any suitable scented oil may be employed without departing from the spirit of my invention or sacrificing its advantages.

Having fully described my invention, what I claim as new and desire to secure by 10 Letters Patent, is:—

1. A composition of the class described containing silver nitrate, camphor, a cyanide solution and whiting.

2. A composition of the class described 15 containing silver nitrate, camphor, sodium cyanide and Paris white.

3. A composition of the class described containing silver nitrate, camphorated wa- 20 ter, sodium cyanide, Paris white and a per- fumed oil.

4. A silver plating solution of the class described composed of pure silver metal dissolved in silver nitrate, camphor gum dissolved in water, sodium cyanide and Paris 25 white.

5. A silver plating solution of the class described composed of pure silver metal dissolved in silver nitrate, camphor gum dissolved in water, sodium cyanide, Paris 30 white and an oil of mirbane.

6. A silver plating solution of the class described made from a solution of camphorated water and silver nitrate, and a solution of sodium cyanide and camphorated water 35 and to the combined solutions is added Paris white.

7. A silver plating solution of the class

described made from a solution of camphorated water and silver nitrate, a solution of sodium cyanide and camphorated water and 40 to the combined solutions is added Paris white and a suitable perfuming oil.

8. A silver plating solution of the class described containing in proportion four hundred and eighty grains of silver nitrate, 45 eight quarts of camphorated water, one and one-quarter pounds of sodium cyanide, ten pounds of Paris white and two teaspoonsful of oil of mirbane.

9. A composition of the class described, 50 containing silver nitrate, camphor, water, sodium cyanide and whiting.

10. A silver plating solution of the class described, containing in proportions, approx- 55 imately four-hundred and eighty grains of silver nitrate, eight quarts of camphorated water, one and one-quarter pounds of sodium cyanide and ten pounds of Paris white.

11. A silver plating solution of the class described, containing in proportions, approx- 60 imately four-hundred and eight grains of silver nitrate, eight quarts of camphorated water, one and one-quarter pounds of sodium cyanide, ten pounds of Paris white, and two teaspoons of a perfuming oil. 65

In testimony that I claim the foregoing as my invention I have signed my name in presence of the subscribing witnesses this first day of June, 1922.

LINDOLPH MINOR SHEROW.

Witnesses:

THOMAS G. BARNES,  
G. S. PURDY.